

## UNITED STATES PATENT OFFICE

2,470,935

## ALLOY ADDITION AGENTS

Arthur Linz, New York, N. Y., assignor to Climax Molybdenum Company, New York, N. Y., a corporation of Delaware

No Drawing. Application September 3, 1947,  
Serial No. 772,011

7 Claims. (Cl. 75—27)

1

The present invention relates to new and useful improvements in alloy addition agents.

Objects and advantages of the invention will be set forth in part hereinafter and in part will be obvious herefrom, or may be learned by practice with the invention, the same being realized and attained by means of the steps, instrumentalities and combinations pointed out in the appended claims.

The invention consists in the novel steps, compositions and improvements herein shown and described.

Heretofore, many different addition agents have been proposed for the addition of alloying elements, such as molybdenum, chromium, tungsten, vanadium to ferrous alloys. Among such addition agents are the ferro-metal agents, such as ferro-molybdenum and ferro-chromium, briquettes formed from the metal oxide and a reducing agents, such as ferro-silicon, silicon, aluminum, calcium silicide and other reducing metals or carbon, bound together with a binder which may be a carbonaceous material such as pitch. Many of these addition agents are relatively expensive to produce, while others introduce a relatively large amount of foreign matter into the alloy and which may appear in the finished alloy as inclusions of slag, while other addition agents give a poor recovery of the alloying metal in the finished alloy and are thus relatively expensive to use.

The present invention has for its object the provision of a novel and improved alloy addition agent which can be produced with very little expense beyond the cost of the alloying metal contained in the addition agent, does not require elaborate equipment for their production, gives good recovery of the alloying metal in the finished alloy, can be used without radical change in alloying technique, and does not result in the addition of abnormal large amounts of foreign material such as slag-forming ingredients. The invention has for a further object the provision of novel and improved alloy addition agents which are economical to produce, are economical to use, are of general application and give excellent results in use.

In accordance with the present invention the alloying addition agent comprises a proportioned mixture of an oxide of the alloying metal to be added to the ferrous alloy and a reducing agent comprising a stable form of calcium carbide, which agent may be formed into convenient briquettes by briquetting under powerful pressure with or without a carbonaceous binder,

2

or may be merely packaged in bags of convenient size or in packages and added to the molten iron or steel in the ladle or otherwise as desired. Calcium carbide, as such, is not suitable for use in such alloying addition agents as the calcium carbide contained therein is so unstable and when briquetted, there is a danger that the briquettes will explode or disintegrate due to the accumulation of gas therein caused by the decomposition of the carbide. However, the calcium carbide reducing agent may be economically and effectively protected against premature decomposition without deleteriously affecting its reducing action on the metallic oxide or the effect of the alloying addition agent as a whole on the ferrous alloy to be produced.

In accordance with the present invention this protection is afforded by treating the calcium carbide particles, whether lumps, grains or dust, with a waterproofing material which is preferably a film-forming material and is in itself a reducing agent and generally a binder of sufficient adhesive force to materially assist in holding the metallic oxide and calcium carbide in intimate contact until the reducing action takes place. The quantity of binder used is from about 1% to about 5% based on the weight of the calcium carbide, and the amount of calcium carbide is generally approximately the stoichiometric quantity required to convert the oxygen of the metallic oxide into carbonmonoxide.

Suitable stabilizing agents for the calcium carbide are crude petroleum, refined mineral oil, paraffin and other mineral waxes, drying and non-drying vegetable oils, rosin, asphalt, still pitch, all of which are film-forming and waterproofing carbonaceous materials which in themselves can serve as reducing agents of a mild kind for the metallic oxide. Other carbonaceous reducing agents which are waterproof may also be used, but I prefer to use the petroleum materials, such as crude petroleum, mineral oil or mineral wax, as these materials may be easily applied to the calcium carbide, as by spraying, to completely coat the external surfaces of the calcium carbide particles and serve to impregnate at least the outer portion of the particles sufficiently so that the particles are effectively waterproofed and thus rendered immune to the action of atmospheric moisture, even to the extent that the particles will withstand immersion in water for a considerable period without reacting with the water.

From about 1% to about 5% of the stabilizing agent is added to the calcium carbide, but I

prefer to use about 3% of the stabilizing agent and apply it to the calcium carbide by spraying it on the carbide at that rate, care being taken that the particles are substantially completely coated with the stabilizing material.

Examples of the metal oxides suitable for use in the alloy addition agents of the present invention are the various oxides of chromium, molybdenum, tungsten, vanadium, comprising the ferrous-alloying metals of the fifth, and sixth periodic groups. These oxides include the trioxide and all the lower oxides of molybdenum, the trioxide and lower oxides of chromium, tungsten trioxide and its lower oxides, and the pentoxyde and the lower oxides of vanadium, some of which are not ordinarily desirable in view of their relative high cost on the basis of the metal contained in them.

Impure oxides, usually in the form of ores of the alloying metals are useful and may be mixed directly with the stabilized calcium carbide without preliminary reduction or extensive chemical treatment of the ore, the ore of course being concentrated to remove from it most or all of the mechanically separable impurities and other undesirable impurities such as sulfur. Among the natural impure oxides which are useful are the following: wolframite, scheelite, hubnerite and ferberite. Of course, many ores may contain impurities which are undesirable from one point of view or another, such as lead, sulfur, arsenic, tin and the like, and the choice of such naturally impure oxides will be determined by the effect of the impurities on the eventual alloy.

In the event that a more active reducing agent is desired than that furnished by the stabilized calcium carbide alone, a portion of the stabilized calcium carbide may be replaced with a more high active reducing agent such as silicon, ferrosilicon, aluminum, magnesium or calcium silicide the amount of such more active reducing agent being less than one-quarter of the total amount of reducing agent.

Where molybdenum trioxide is used as the metallic oxide, 144 pounds of it are mixed with about 75 pounds of the stabilized calcium carbide and preferably formed into briquettes which are added in the desired quantity to the molten iron or steel in the ladle. Under the heat of the molten metal, the oxide is reduced according to the equation:



If molybdenum dioxide is used, 384 pounds of it are mixed with about 75 pounds of the stable calcium carbide and the reaction proceeds according to the equation:



Using about 75 pounds of the stable calcium carbide in each of the following instances, the equations are:

Using 232 pounds of tungsten trioxide



Using 150 pounds of vanadium sesquioxide



Using 166 pounds of chromite, calculated as pure  $\text{FeCr}_2\text{O}_4$



In each instance it will be noted that the quantity of calcium carbide is substantially the quantity needed on a stoichiometric basis to convert the metallic oxide into metal with the resulting reaction products of carbon monoxide, and lime. The carbonaceous material forming the stabilizing agent for the calcium carbide has been disregarded in the above calculations but introduces no great change in the calculations due to its relatively small quantity.

The invention in its broader aspects is not limited to the specific steps shown and described but departures may be made therefrom within the scope of the accompanying claims without departing from the principles of the invention and without sacrificing its chief advantages.

What is claimed is:

1. A self-reducing alloy addition agent comprising a mixture of an oxide of a metal selected from the group consisting of molybdenum, chromium, tungsten and vanadium, and calcium carbide, said particles of calcium carbide being stabilized by a coating of a waterproofing carbonaceous material which acts as a reducing agent for the metal oxide.

2. A composition as claimed in claim 1 in which the quantity of stabilized calcium carbide is approximately the quantity necessary to reduce the metal oxide with the formation of lime and carbon monoxide.

3. A composition as claimed in claim 2 in which the calcium carbide is stabilized by coating the particles with a substantially nonvolatile petroleum oil.

4. A composition as claimed in claim 1 in which the calcium carbide is stabilized by coating the particles with a substantially nonvolatile petroleum oil.

5. A composition as claimed in claim 1 in which the metal oxide is a molybdenum oxide.

6. A composition as claimed in claim 1 in which the metal oxide is a chromium oxide.

7. A composition as claimed in claim 1 in which the metal oxide is chromite.

ARTHUR LINZ.

#### REFERENCES CITED

The following references are of record in the file of this patent:

#### UNITED STATES PATENTS

| Number    | Name   | Date           |
|-----------|--------|----------------|
| 866,562   | Becket | Sept. 17, 1907 |
| 1,275,449 | Lemon  | Aug. 13, 1918  |